

## UNITED STATES PATENT OFFICE

2,104,169

NONAGING FLAT SILICON STEEL STRIP AND  
METHOD OF PRODUCING THE SAMECharles A. Scharschu, Brackenridge, Pa., assignor  
to Allegheny Steel Company, a corporation of  
PennsylvaniaNo Drawing. Application August 3, 1933,  
Serial No. 683,476

## 14 Claims. (Cl. 148—12)

My present invention relates to a method of annealing cold rolled silicon steel strip to make it flat and non-aging.

The general practice has been to box anneal the finished cold rolled silicon steel strip at temperatures between 1400° and 2000° F. in coils and slowly cool to obtain good magnetic properties and a product which is non-aging. Strip of this nature which has been given a final anneal in coils unavoidably takes the "set" of the coil and such strip will not thereafter lie flat so that punchings or laminations made from coils annealed in this manner will be curved or non-flat, thus having a low space factor which makes it difficult and sometimes impossible to get the proper weight of punchings or laminations into a core, and even when the prescribed weight can be obtained considerable strain is introduced into the punchings themselves, when the cores are tightened, which adversely affects the magnetic qualities. Again, finished strip which has been annealed continuously in strip form wherein the strip is subjected to the above annealing temperatures for a comparatively short time and cooled at a fairly rapid rate may be flat, if the rolling and annealing operations have been conducted in a proper manner, but in such case the magnetic properties are not permanent. Consequently, in service, it has been found that the watt loss values will increase and the permeability will decrease and hence electrical apparatus built up from strip which has been so treated will lose a considerable part of its efficiency. In addition, strip which has been so treated does not possess the well known non-aging properties which are characteristic of silicon steels and tests have shown that the watt loss values of steel so treated will increase from 25 to 50% when subjected to a temperature of 210° F. for 600 hours.

It is accordingly one of the objects of the present invention to provide cold rolled silicon steel strip which is not subject to the defects and disadvantages above outlined and to provide a method of producing such silicon steel.

It is another object of the invention to provide cold rolled silicon steel strip which is characterized by having been subjected to a final anneal of the character to be set forth whereby the indicated properties are provided in such steel strip.

A further object of the invention is to subject fully annealed cold rolled silicon steel strip to a final annealing operation under such conditions as will ensure production of such steel with the desired flat and non-aging properties.

A still further object is to subject cold rolled silicon steel strip to a final anneal at 1000 to 1300° F. in the manner of a continuous anneal for a suitable length of time and suitably cooling the so annealed strip.

Other and further objects and advantages will be understood by those skilled in the handling of silicon steel or will be apparent or pointed out hereinafter.

In general, my present invention comprises the subjection of cold rolled silicon steel strip which has been either box annealed or continuously annealed at a temperature between 1400 and 2000° F. to a final annealing operation. My annealing operation is carried out at 1000 to 1300° F., preferably at about 1100° F., in the manner of a continuous anneal for two to three minutes or for a length of time necessary to produce flat and non-aging characteristics in the precise material undergoing treatment and then either rapidly or slowly cooling the same.

In order that my invention might be better understood it might be well to describe the process by which the cold rolled silicon steel strip is produced.

The silicon steel ingots are heated to a suitable temperature and hot rolled into strip of as light a gauge as possible, that is, to a thickness which is generally from .100 inch to .045 inch depending upon the silicon content, the kind and type of mill used, and the size of the reducing rolls of the mill. The hot rolled strip is generally coiled and then annealed and pickled. The annealed and pickled strip is then reduced by cold rolling to the finished gauge. Usually the cold rolled strip is annealed before the finished gauge is reached, in order to obtain the best magnetic properties. When the strip has been cold rolled to the finished gauge it is again coiled and the coil is then either box annealed at a temperature between 1400 to 2000° F. and then slowly cooled, or the strip is uncoiled and continuously passed while flat through a furnace maintained at a temperature within the above temperature range. It is well known that strip which has been box annealed is non-aging, but will take the set of the coils, and when reeled from the coil will not be flat, and has the disadvantages which have already been pointed out.

It has been found that exceptionally good magnetic results may be obtained by the method of continuous annealing, but when the strip has been annealed in this manner it is aging, and when used in electrical apparatus the watt loss will increase and the permeability decrease to such an

extent that the apparatus is no longer efficient. In order to render such material non-aging it is customary to anneal the strip for a long time within the temperature range given above and to slowly cool. However, when this annealing is carried out in the coil the strip will no longer be flat and when used in electrical apparatus inferior results will be obtained as described above.

The above is descriptive of the methods which are commercially used to produce silicon steel strip of a commercial grade, and in no way relates to my invention.

I have discovered that when silicon steel strip which has been box annealed in coils within the temperature range given above is uncoiled and subjected to a continuous anneal while flat and at a temperature between 1000 to 1300° F. and then rapidly cooled such strip will be perfectly flat and will have magnetic properties equal to or slightly better than the box annealed strip, and that these values will be permanent. Such strip can then be coiled without taking coil set. In other words, the strip when uncoiled is flat and is non-aging. I have also found that when silicon steel strip which has been continuously annealed within the temperature range of 1400 to 2000° F., is then subjected to a continuous anneal between 1000 and 1300° F. for a few minutes and rapidly cooled, it will be flat and non-aging, and have magnetic properties equal to or slightly better than those obtained in the first anneal. Such strip may also be coiled without taking a coil set.

The silicon steel of the present invention may contain from about .5 to about 4.50% silicon and more broadly stated contains less than about 5% silicon. In general, the strip steel is intended for use in electrical apparatus such as transformers, motors and other electrical equipment making use of so-called electrical steels and is particularly suitable for punchings or laminations for use therein.

Since the material of this invention is strip material produced by hot and cold rolling procedures, the rollings both hot and cold are carried on in the usual manner of producing strip material that is, all of the rolling is carried on in one direction, the direction in which the ingot is rolled.

#### Example I

50 Silicon steel strip containing about .93% silicon and .018 inch thick after box annealing in the regular manner had a watt loss of 1.009 watts per pound at 10,000 B and 60 cycles. After such box anneal the strip was very wavy and would not lie flat. The strip was then uncoiled and while flat was annealed continuously at about 1100° F. for about two to three minutes and then rapidly cooled while still flat. When cooled after this latter anneal the strip was perfectly flat and did not take a set when recoiled. Tests showed that it had a watt loss of only .993 watt per pound at 10,000 B and 60 cycles. After aging 1150 hours at 210° F. the watt loss value was about 1.013 watts per pound at 10,000 B and 60 cycles indicating that no aging had resulted.

#### Example II

70 Silicon steel strip of a thickness of .024 inch and having a silicon content of about 2.60% silicon after box annealing in the regular manner had a loss of 1.228 watts per pound at 10,000 B and 60 cycles. After this treatment the strip was very wavy and would not lie flat when uncoiled. The strip was then annealed continuously

while flat at about 1100° for about two to three minutes and then rapidly cooled while still flat. After this anneal, the strip was perfectly flat and had a watt loss of 1.098 watts per pound at 10,000 B and 60 cycles. After aging 1150 hours at 210° F. the watt loss value was 1.108 watts per pound at 10,000 B and 60 cycles indicating that no aging had resulted.

I have accordingly discovered that by subjecting silicon steel strip of the character set forth to a final anneal, subsequent to the normal final anneal, under the conditions specified, I can produce flat non-aging cold rolled silicon steel strip of reduced watt loss and permanent magnetic properties.

Such strip is far more valuable and has much greater utility and uniformity in electrical apparatus than cold rolled silicon steel strip made by the present methods known to me.

It is understood that the foregoing is intended more in an illustrative manner than in a limitative manner and that suitable additions, omissions, variations and substitutions may be made without departing from the spirit and scope of the invention.

What I claim as new and desire to secure by Letters Patent is:

1. In a method of making magnetic material in the form of silicon steel strip, the steps which consist in casting a steel ingot having a silicon content of from about .5% to 5%, in reducing the ingot by hot rolling to a strip of intermediate gauge, in annealing the hot rolled strip, in pickling the annealed strip, in cold rolling the pickled strip to finished gauge, in annealing the strip of finished gauge within a temperature range of from 1400-2000° F., in then cooling the strip, then in continuously annealing the strip while flat at a temperature of from 1000 to 1300° F., and then in cooling the strip.

2. In a method of making magnetic material in the form of silicon steel strip, the steps which consist in casting a steel ingot having a silicon content of from about .5% to 5%, in reducing the ingot by hot rolling to a strip of intermediate gauge, in annealing the hot rolled strip, in pickling the annealed strip, in cold rolling the pickled strip to finished gauge, in annealing the strip of finished gauge within a temperature range of from 1400-2000° F., in then cooling the strip, then in continuously annealing the strip while flat at a temperature of about 1100° F., and then in cooling the strip.

3. In a method of making magnetic material in the form of silicon steel strip, the steps which consist in casting a steel ingot having a silicon content of from about .5% to 5%, in reducing the ingot by hot rolling to a strip of intermediate gauge, in pickling the strip, in cold rolling the pickled strip to finished gauge, in box annealing the strip of finished gauge within a temperature range of from 1400-2000° F., in slowly cooling the strip, then in continuously annealing the strip while flat at a temperature of from between 1000 and 1300° F., and then cooling the strip while flat.

4. In a method of making magnetic material in the form of silicon steel strip, the steps which consist in casting a steel ingot having a silicon content of from about .5% to 5%, in reducing the ingot by hot rolling to a strip of intermediate gauge, in cold rolling to finished gauge, in box annealing the strip of finished gauge within a temperature range of from 1400-2000° F., in cooling the strip slowly, then in continuously anneal-

ing the strip while flat at a temperature of about 1100° F., and then in cooling the strip while flat.

5. In a method of making magnetic material in the form of silicon steel strip, the steps which consist in casting a steel ingot having a silicon content of from about .5% to 5%, in reducing the ingot by hot rolling to a strip of intermediate gauge, in cold rolling to finished gauge, in annealing the strip of finished gauge within a temperature range of from 1400-2000° F., in cooling the strip, and then in continuously annealing the strip while flat at a temperature of about 1100° F.

10 6. In a method of making magnetic material in the form of silicon steel strip, the steps which consist in casting a steel ingot having a silicon content of from about .5% to 5%, in reducing the ingot by hot rolling to a strip of intermediate gauge, in cold rolling to finished gauge, in box annealing the strip of finished gauge within a temperature range of from 1400-2000° F., in cooling the strip slowly, then in continuously annealing the strip while flat at a temperature of from 1000 to 1300° F., and then in rapidly cooling the strip while flat.

15 7. In a method of making magnetic material in the form of silicon steel strip, the steps which consist in effecting a heavy reduction by cold work, heating the strip to a temperature of from about 1400 to about 2000° F., in cooling the strip, then subjecting the strip while flat to a continuous anneal of from about 1000° to about 1300° F., and then cooling the strip while flat.

20 8. In a method of making magnetic material in the form of silicon steel strip, the steps which consist in effecting a heavy reduction by cold work, heating the strip to a temperature of from about 1400 to about 2000° F., in then cooling the strip, then subjecting the strip while flat to a continuous anneal at about 1100° F., and then in cooling the strip while flat.

25 9. In the art of making a coil of magnetic material in the form of silicon steel strip which is non-aging and free from coil set, the steps which consist in reducing suitable silicon steel by hot and cold rolling operations to a strip of final gauge, in then annealing such strip of final gauge within a temperature range of from 1400 to 2000° F., in cooling the strip, in continuously annealing the strip while flat within a temperature range of from 1000 to 1300° F., in then cooling the strip while flat and then in coiling the same.

30 10. In the art of making a coil of magnetic material in the form of silicon steel strip which is non-aging and free from coil set, the steps which consist in reducing suitable silicon steel

35 by hot and cold rolling operations to a strip of final gauge, in coiling the strip of final gauge, in box annealing the coiled strip, in cooling the coiled strip, in uncoiling the strip, in continuously annealing the strip while flat within a temperature range of from 1000 to 1300° F., in cooling the strip while flat and then in re-coiling the strip.

40 11. In the art of making a coil of magnetic material in the form of silicon steel strip which is non-aging and free from coil set, the steps which consist in reducing suitable silicon steel by hot and cold rolling operations to a strip of final gauge, in then annealing such strip of final gauge within a temperature range of from 1400 to 2000° F., in cooling the strip, in continuously annealing the strip while flat at about 1100° F., in then cooling the strip while flat and then in coiling the same.

45 12. In the art of making a coil of magnetic material in the form of silicon steel strip which is non-aging and free from coil set, the steps which consist in reducing suitable silicon steel by hot and cold rolling operations to a strip of final gauge, in coiling the strip of final gauge, in box annealing the coiled strip, in cooling the coiled strip, in uncoiling the strip, in continuously annealing the strip while flat at about 1100° F., in cooling the strip while flat and then in recoiling the strip.

50 13. As a new article of manufacture, a coil of magnetic material in the form of cold rolled silicon steel strip having a silicon content between approximately .5% and 5% which is non-aging and free from coil set and produced from a strip of silicon steel having a silicon content within the limits set forth which has been annealed at a temperature between approximately 1400° F. and 2000° F., cooled, then subjected to a continuous anneal at a temperature of approximately 1100° F. and again cooled.

55 14. As a new article of manufacture, non-aging magnetic material in the form of silicon steel strip free from coil set and having a silicon content between approximately .5% and 4.5% and produced from silicon steel strip having a silicon content within said range which has been subjected to hot and cold roll reductions, then annealed at a temperature between approximately 1400° F. and 2000° F., cooled, then given a continuous anneal while flat at a temperature between approximately 1000° F. and 1300° F. and then again cooled.

CHARLES A. SCHARSCHU. 55